

March 22, 1938.

J. F. McNUTT

2,111,897

METHOD OF APPLYING A DECALCOMANIA

Filed Nov. 16, 1935



Fig. 1



Fig. 2

INVENTOR.

James F. McNutt  
BY  
Huey Brock West

ATTORNEY.

## UNITED STATES PATENT OFFICE

2,111,897

## METHOD OF APPLYING A DECALCOMANIA

James F. McNutt, Cleveland, Ohio, assignor to  
The American Decal Corporation, Youngs-  
town, Ohio, a corporation of Ohio

Application November 16, 1935, Serial No. 50,167

2 Claims. (Cl. 41—33)

This invention relates to a method of applying a design or label to an object or container having a vitreous surface.

One of the objects of the invention is to provide 5 a decalcomania and method of applying the same to an object or container having a vitreous surface which consists essentially in applying to the surface to be decorated a collodion film containing thereon a design containing a pigment and a material which will readily fuse with the surface to be decorated and then firing the object by first heating it slowly and at a uniform rate of increase in temperature until it reaches a temperature of about 450° F.; and then raising the 10 temperature to about 1200° F. at a faster rate of increase and for a sufficient period of time to cause the design to be thoroughly fused with the surface being decorated.

In my Reissue Patent No. 19,839, dated January 28, 1936, I have disclosed a decalcomania and method of making the same. I have found that a design applied as described therein is likely 15 to become injured or destroyed if the object is subjected to too high a temperature at the beginning of the firing operation.

My decalcomania preferably consists of a collodion film attached to a backing strip and to the exposed surface of which is affixed a design containing a pigment and a material which will readily fuse with the surface to be decorated. When the decalcomania is applied to the surface to be decorated, the backing strip is removed and the collodion film applied to the surface to be decorated. The object is then fired to cause the design to be fused with such surface. If the object is fired at too high a temperature at the beginning, or if the temperature is increased too rapidly, the collodion film may be consumed too rapidly 20 or sufficiently rapid oxidation may take place to injure or destroy the design. The object should be first fired at a sufficiently low temperature and at a sufficiently low rate of increase in temperature that the film will be consumed or volatilized without injury to the design. The temperature of 25 the object being fired should preferably not exceed about 450° F. during the first hour of the firing operation. If this precaution is taken, the film will be consumed without injury to the design and the design will adhere to the surface to be decorated and become fused with such surface upon further heating at a higher temperature. The temperature required to effect a proper 30 fusing is usually between 1100° and 1200° F. or

slightly below the fusing point of the surface to be decorated.

Further and more limited objects of my invention will appear as the description proceeds and by reference to the accompanying drawing in 5 which Fig. 1 is a somewhat graphic illustration indicating the preferred manner in which the object should be fired and Fig. 2 is a sectional view of a label or decalcomania before it is applied to the surface to be decorated, the thickness 10 being greatly exaggerated.

Referring now to the drawing the decalcomania consists essentially of a backing strip 1 formed of suitable flexible material such as 15 paper and to which is secured a collodion film 2 which is held thereon preferably by means of a water soluble mucilaginous paste 3. The reference character 4 designates the design which is carried by the exposed surface of the collodion film and the reference character 5 designates a 20 layer of finely divided particles of ground glass or silica which covers the design and which when subjected to heat forms a smooth, thin, transparent covering for the design.

According to the preferred method of applying 25 the decalcomania to the surface to be decorated, the decalcomania prepared preferably as described in my copending application hereinbefore referred to, is soaked in water for a sufficient 30 period of time to soften it and to facilitate its application to the surface to be decorated. The decalcomania is then placed over the bottle or other surface which is to be decorated with the backing strip contiguous to such surface and the 35 design outermost. As the decalcomania has been soaked in water for some time, the water soluble mucilaginous paste is softened and the backing strip may be readily removed, leaving only the collodion film with the design thereon and having 40 on the reverse side thereof a very small amount of adhesive material which enables the film to stick on the surface to be decorated and eliminates the necessity for first coating such surface with a varnish. As this backing strip is removed the collodion film is pressed into contact 45 with the surface to be decorated. The thickness of this collodion film is such that it may be handled or moved around on the surface of the bottle if it is not located in the proper position. The bottle with the decalcomania applied thereto 50 is then placed in a kiln or other suitable retort heated in any suitable manner. According to the preferred method of practicing the invention I fire the object by slowly raising the temperature 55

for the first hour and at a uniformly increasing rate until it reaches a temperature of about 450° F. The temperature is preferably gradually increased at the rate of about 7.5° F. per minute 5 until a temperature of about 450° F. is reached. After this temperature is reached the object may be heated either rapidly or slowly and at any desired rate of increase until a temperature between 1100° and 1200° F. is reached, depending upon the 10 nature of the object being decorated. This usually requires about an hour in order to thoroughly fuse the design with the surface being decorated. As the object is first heated slowly and at a uniformly increasing rate, the collodion film will be 15 consumed or volatilized without producing a flame or sufficiently high temperature to injure or destroy the design, that is, the pigment and vehicle. The design will adhere to the surface being decorated and the film will be entirely consumed. The letters or designs forming the label 20 penetrate the body being decorated and become thoroughly and permanently fused and integrated therewith. The outer layer of material on the collodion film also fuses with the object and forms 25 a thin, smooth, transparent film over the surface of the design or label and it is impossible to remove the design or label thus applied by any means whatsoever without destroying the identity of the object or design. 30 The particular "ink" and the particular manner of forming the design on the collodion film form no part of this invention and are described in my copending application hereinbefore referred to. 35 It will now be clear that I have provided a method of applying a design or label to an object having a vitreous surface which will accomplish the objects of the invention as hereinbefore stated. It is, of course, to be understood that the 40 embodiment of the invention herein disclosed is merely illustrative and is not to be considered in a limiting sense. It is also to be understood that I do not limit myself to any particular "ink" or mixture of vehicle and pigment as various 45 mixtures and colors or combination of colors and designs may be used depending upon the exigencies of the occasion and the nature of the par-

ticular object being decorated. In the specification and claims I refer to the film of material to which the design is applied as a "collodion film". By this term I mean to include any material of a similar nature or foundation which is 5 homogeneous and non-fibrous, such as cellulose nitrate, cellulose acetate, celluloid, viscose or pyroxylin, but to exclude such material as paper. It is also to be understood that the particular rate of increase in temperature illustrated in 10 the drawing may be varied slightly depending upon the particular nature of the object being decorated although I have found that the best results are obtained if the object is fired substantially as described although the invention is limited only in accordance with the scope of the 15 appended claims.

Having thus described my invention, what I claim is:

1. The method of applying a decalcomania to 20 an object having a vitreous surface which consists in applying to such surface a collodion film having a design thereon containing a pigment and a material that will readily fuse with the surface to be decorated, then firing the object by 25 heating it first at a sufficiently low temperature and at a sufficiently low rate of increase in temperature to cause the film to be consumed and the design to become attached to such surface without injury to the design and then heating 30 it at a sufficiently high temperature to thoroughly fuse the design with such surface.

2. The method of applying a decalcomania to a vitreous fusible surface which consists in applying to such surface a collodion film having 35 a design formed thereon containing a pigment and a material which will readily fuse with the surface to be decorated, then heating the surface and film to about 450° F. at a sufficiently low rate of increase in temperature to cause the 40 film to be consumed and the design to become attached to such surface without injury to the design and then progressively increasing the temperature of the surface being decorated to between 1100° F. and 1200° F. to thoroughly fuse 45 the design with such surface.

JAMES F. McNUTT.